

Feb. 13, 1934.

A. E. NOBLE

1,946,498

## ELECTRIC DISCHARGE DEVICE

Filed Nov. 15, 1929



## FIG.2.



### Inventor

Aubrey E. Noble

By his Attorneys

By his Attorneys  
Dollebeek & Ledbetter

## UNITED STATES PATENT OFFICE

1,946,498

## ELECTRIC DISCHARGE DEVICE

Aubrey E. Noble, Lynbrook, N. Y., assignor to  
 Claude Neon Lights, Inc., New York, N. Y., a  
 corporation of New York

Application November 15, 1929

Serial No. 407,413

2 Claims. (Cl. 176—122)

The present invention relates to a gaseous discharge luminous tube device containing a gas filling and adapted to emit light upon the discharge of electricity through the said gaseous filling. The said invention relates more particularly to such a device in which the rare gas employed is relatively active, as for example, helium. When a gas such as helium is employed as the path of an electric discharge between electrodes, as for example, iron, copper or nickel electrodes, the helium tends to be relatively rapidly destroyed so far as its capacity to conduct the current and emit light is concerned, probably due to mutual action between the gas and the cathode. Among the rare gases, this tendency is more pronounced in helium than in the others and in this sense the helium is herein characterized as active. For this reason, a gaseous discharge device which depends for the most part upon helium for its effect, has ordinarily a relatively very short life. For example, a tube containing helium at a pressure of 3 to 5 millimeters with an ordinary copper electrode has in general a very short effective life which may be, for example, 2 to 30 hours, under the influence of an electric discharge. The effective life or duration of a device of this character may be measured by passing an electric discharge through it having the requisite voltage and current characteristics necessary to cause the emission of light and observing the elapsed time between the beginning of the emission of light and the cessation thereof.

By increasing the total amount of the gas in the discharge device, as for example, by increasing the pressure of the helium to 10 to 15 millimeters, the life of the device may be greatly increased, as for example, to 1500 hours. This life however, is not sufficiently long to meet commercial demands and is attained by the sacrifice of energy and luminous efficiency inasmuch as the potential drop per unit length of gas column of a given diameter, such as 11 to 15 millimeters, is much greater at pressures corresponding to 10 to 15 millimeters of mercury, than is the case at lower pressures such as 3 to 5 millimeters of mercury.

The present invention provides a discharge device containing helium or other relatively active gas which not only has an unusually long life, but is also adapted to operate at a high efficiency, that is to say, at such pressures that a maximum length and therefore volume of gas column may be energized by a given electric potential. This high efficiency is secured by operating between certain limits of pressure of the gaseous filling, which in the case of helium is in the neighbor-

hood of 3 to 5 millimeters as measured in terms of mercury in the usual way, for a tube having a diameter of 11 to 15 millimeters. The term high efficiency means and relates to that luminous efficiency which is produced by operating at or between certain limits of pressure as herein described, and the term high efficiency is to be taken as having this meaning. Notwithstanding the use of small quantities of helium as measured by small and therefore highly efficient pressures from the point of view of high luminous efficiency, the invention provides a luminous device having a greatly increased life.

The invention comprises the combination of rarified helium under certain optimum pressure conditions in combination with discharge electrodes comprising a stabilized cathode. The cathode may be iron, copper, nickel, carbon or other refractory conducting substance stabilized by treatment which provides it with a coating comprising a suitable oxide of an electro-positive metal or derivative thereof.

The suboxides of electro-positive metals appear to be particularly desirable. These may be produced by providing a refractory electrode such as copper with a coating comprising a suitable oxygen compound such as the oxide, hydroxide or peroxide of an electro-positive metal, as for example, barium peroxide, and then subjecting such coated electrode to heat to bring about reaction to form decomposition or reduction products such as the suboxide of the active material, as for example barium suboxide. The term suboxide as used herein includes the products produced when peroxides are thermolyzed or subjected to decomposition by heat to yield a lower oxide or suboxide.

The preparation of the stabilized electrode or cathode may be carried out as follows. The electrode is coated upon the inside thereof with a coating comprising barium peroxide and is then subjected to heat whereupon the peroxide decomposes. The decomposition or thermolytic products comprise what is herein termed barium suboxide and the resulting product forms a particularly stable electrode or cathode and one which in combination with the gas filling such as helium provides a discharge device having an unusually long life such as three thousand hours or more.

Instead of the suboxide of barium, the suboxides of other electro-positive elements may be employed, particularly elements of the alkaline earth group such as calcium and strontium.

Instead of stabilizing the cathode with oxides

as hereinabove described, stabilization at least to some extent, may be carried out by means of strongly electro-positive elements including those of the alkali group, as for example, potassium, 5 caesium and the like. For example, a gaseous discharge device with a rarified helium filling at a pressure of 3 to 5 millimeters may be equipped with an anode and a cathode, the latter being provided with metallic caesium as a coating. By 10 this means, a tube may be provided which comprises a combination of helium adapted to operate at a high energy efficiency with a stabilized cathode and possessing a moderate life, as for example, 340 hours.

15 Stabilization by means of alkali metals is therefore not as effective as stabilization by means of oxides as hereinabove described.

16 The invention will be described in greater detail with reference to the accompanying drawing 20 which illustrates one embodiment thereof and in which

Figure 1 represents a gaseous discharge luminous tube containing rarified helium at a pressure of 3 to 5 millimeters and provided with stabilized electrodes intended for use with alternating current and

Figure 2 represents one of the electrodes in detail.

25 The gaseous discharge tube 1 which may have a length, between electrodes, of 17 feet and a diameter of 11 millimeters may be formed in any desired shape such as the U-shape shown in Figure 1 and is provided at each end with electrodes 2 which may in the event that alternating current is employed, be identical in form and structure inasmuch as under these conditions each electrode acts alternately as cathode and anode. The electrodes are as shown connected to the secondary 3 coil of a transformer, the primary 4 of 30 which is adapted to be supplied with current from the generator 5. The tube 1 may be made of yellow glass and in this event is adapted to produce a decidedly yellow light. The pressure of the helium filling in the tube is carefully adjusted 35 to correspond with that pressure at which the efficiency is at a maximum. This pressure may be for example 4 millimeters of mercury as measured in the usual way. As already described, the invention comprises the combination of helium at 40 pressures adapted to produce high energy and luminous efficiency acting in conjunction with electrodes stabilized so that the combination yields a device having a remarkably long life.

45 A stabilized electrode is shown in enlarged view partly in section in Figure 2. It consists of a nickel cylinder 2 closed at one end and provided on the inside with a coating 6 comprising the thermolyzed products of a peroxide such as barium peroxide.

50 The operation of the invention is carried out as follows:

55 The tube having been provided with a helium filling and stabilized electrodes as shown is connected to the secondary of a transformer through

the lead wires 7 and 8 and a discharge current of for example, 25 milliamperes, is supplied to the tube at a potential of 15,000 volts, for example. The operation in this manner causes the emission of a yellow or tan light when helium is employed as filling and may be continued for a period of 3,000 hours or more.

60 To recapitulate, the invention comprises, in combination, a gas filling in an electric discharge luminous tube device at pressures corresponding to high energy and luminous efficiency and a cathode or electrodes treated in such a manner that notwithstanding the activity of the gas and the relatively small quantity of gas employed, the cooperation between the electrode and the gas is such that high energy efficiency combined with long effective life is secured. The specific active gas preferred is helium and where helium is employed, the present invention provides a luminous tube discharge device adapted to yield light of a 65 yellowish or tan color.

70 The invention furthermore comprises the combination of the features herein disclosed with a transparent yellow envelope such as yellow glass, whereby a very efficient long life yellow light may 100 be obtained.

75 The advantages of the invention have been set forth in some detail and the preferred embodiments have been described. It is to be understood, however, that various changes may be 105 made without departing from the invention or sacrificing any of the advantages enumerated, or any other advantageous results which may be attained by an application of the principles and facts set forth.

80 To summarize, it will be noted that by employing helium at that relatively low pressure which corresponds approximately to a minimum potential drop through the gas column with respect to the internal diameter of the tube and in combination 110 with an activated oxide cathode, that a long life high efficiency helium light is obtained, notwithstanding the relatively low helium pressure. When, furthermore, a yellow envelope is used, a 115 long life helium luminescent tube emitting light of 120 a decidedly yellow color is obtained.

85 What I claim is:—

1. A luminescent tube adapted to emit yellow light comprising an envelope transparent to yellow rays and having an external diameter of the 125 order of 11 to 15 millimeters, a filling of helium at a pressure of the order of 3 to 5 millimeters and a cold cathode comprising the decomposition products of an alkaline earth oxygenated compound.

2. A positive column gaseous discharge tube which emits yellow light throughout a period of useful commercial life which comprises an envelope of yellow glass, a principal filling of helium, and a cold cathode comprising the decomposition 130 product of a compound of an alkaline earth metal and oxygen.

AUBREY E. NOBLE.